

July 2, 1929.

J. E. ANCHONDO

1,719,794

IGNITING TIP FOR CIGARS AND CIGARETTES

Filed March 30, 1927

*Fig.1.*



*Fig.2.*



*Fig.3.*



INVENTOR  
*Juan E. Anchondo*,  
BY

*Philip E. Sizemore*,  
ATTORNEY

## UNITED STATES PATENT OFFICE.

JUAN E. ANCHONDO, OF TUCSON, ARIZONA.

## IGNITING TIP FOR CIGARS AND CIGARETTES.

Application filed March 30, 1927. Serial No. 179,552.

My invention aims to provide an improved match substance adapted to be applied to cigarettes, cigars and the like and a scratching surface therefor.

Various match substances heretofore proposed for use on self-ignited cigarettes and cigars have included ingredients such as white or red phosphorous, which are injurious to the smoker. White phosphorous, upon oxidation, emits a poisonous fume which, in a short time, causes necrosis of the bones, particularly of the teeth and jaws of the smoker. Red phosphorus is non-poisonous but it changes to white phosphorus at a temperature of 536° F., or when it is subjected to the heat of ignition and, hence, it is objectionable also because of its toxic effect. Also, many of the old match substances are difficult to scratch, and burst into a flame emitting toxic fumes.

One of the objects of my invention is to provide an easily ignitable match composition that will not burst into a flame when it is ignited and that will not give off toxic fumes which are dangerous for a smoker to inhale.

Other objects of my invention appear in the specification when considered in connection with the illustrative example thereof shown in the accompanying drawing, where-

Fig. 1 is a side view of a cigarette having my improved match composition applied to one end;

Fig. 2 is a view corresponding to Fig. 1 but showing the match end in section; and

Fig. 3 is a perspective view on a reduced scale of a cigarette package having a scratching surface adapted to ignite the match substance.

Referring particularly to the drawing, I have shown a cigarette 10 having a match tip 11 composed of my improved self-igniting substance and being applied thereto while it is in a plastic state.

My improved composition comprises a mixture of a suitable tinder, an ignition producing substance, a filler and an adhesive. I use pulverized charcoal or fine sawdust as the tinder; chlorate of potassium or sodium as the igniting substance; powdered clay or infusorial earth as the filler; and any suitable glue or vegetable gum as the adhesive or binding agent.

One satisfactory formula for my substance includes charcoal, chlorate of potassium, powdered clay and a mucilage of vegetable gum mixed in the following proportions:

|                                 |          |    |
|---------------------------------|----------|----|
| Chlorate of potassium or sodium | 15 parts | 60 |
| Charcoal                        | 6 parts  |    |
| Powdered clay                   | 3 parts  |    |
| Vegetable gum                   | 1 part   |    |

The charcoal, in combination with the other ingredients, is intended to hold the coal of fire after ignition takes place to insure proper lighting of the cigarette under the most unfavorable conditions.

The chlorate of potassium or sodium is the ingredient which, when scratched against a surface coated with phosphorus, produces the spark which causes ignition. The powdered clay not only serves as a filler but tends to prevent flaring up of the flame after ignition and to cause slow burning. In other words, it retards flaming combustion. The glue or vegetable gum, is used as a binder to combine the component parts together and to the ends of cigarettes or cigars.

My improved composition does not include any substance which is injurious to the smoker even if the fumes are inhaled. Moreover, the presence of powdered charcoal in the substance tends to prevent the formation of any dangerous monoxide fumes because the carbon absorbs the oxygen. Further, my substance, when it is ignited, does not flare up and give off objectionable fumes or smoke and, due to its slow burning characteristic produced by the presence of the powdered charcoal and clay, it burns sufficiently long to insure that the cigarette or cigar will be lighted properly. I have found that my substance can be made at a very low cost and only a small amount needs to be used.

Referring to Fig. 3 I have shown a cigarette carton 12 having my improved scratching surface 13 for the convenience of cigarette smokers. I have found that a thin paste composed of phosphorous, preferably red phosphorous, peroxide of manganese and mucilage applied to the surface and then sprayed with a solution of chlorate of sodium or potassium, forms an excellent scratching surface for my match tips, insuring ignition without vigorous scratching.

My match tips, when rubbed slightly on the scratching surface will ignite readily without

breaking off and will burn through to the tobacco and ignite it without the necessity of drawing on the cigarette.

Obviously the present invention is not restricted to the particular embodiment thereof herein shown and described. Moreover, it is not indispensable that all the features of the invention be used conjointly since they may be employed advantageously in various combinations and subcombinations.

What I claim is:

1. An igniting tip for cigarettes and the like composed of chlorate of alkali metal combined with a tinder and a non-combustible filler adapted to burn by forming a live coal without flaring into a flame.
2. A tip for cigarettes and the like composed of a tinder, potassium chlorate, an earthy filler, and an adhesive substance.
3. A tip for cigarettes and the like composed of powdered charcoal, chlorate of an alkali metal, clay and an adhesive substance.
4. An igniting tip for cigarettes and the like composed of powdered charcoal, an alkali

metal chlorate, clay, and an adhesive substance all combined in approximately the following proportions:

|                              |          |
|------------------------------|----------|
| Powdered charcoal            | 6 parts  |
| Potassium or sodium chlorate | 15 parts |
| Clay                         | 3 parts  |
| Adhesive material            | 1 part   |

5. An igniting tip for cigarettes and the like composed of powdered charcoal, chlorate of potassium, powdered clay, and an adhesive substance.

6. In combination with a tip for self-igniting cigarettes and the like composed of powdered charcoal, chlorate of an alkali metal, a combustion retarding ingredient, and a binder, a scratching surface composed of a coating containing red phosphorus, peroxide of manganese, and mucilage sprayed with a solution of a chlorate of an alkali metal.

In testimony, that I claim the foregoing as my own, I have hereto affixed my signature.

JUAN E. ANCHONDO.